

1

3,167,511

## METAL WORKING LUBRICANT

William Crawford, Leigh-on-Sea, and James Arthur Herbert Wood, Fobbing, Essex, England, assignors, by mesne assignments, to Secony Mobil Oil Company, Inc., New York, N.Y., a corporation of New York  
No Drawing. Filed Apr. 13, 1961, Ser. No. 102,675  
1 Claim. (Cl. 252—48.8)

The present invention is concerned with lubricants, especially those intended for metal working applications of all kinds and particularly metal cutting, rolling and drawing. The invention is particularly concerned with an additive for such lubricants which will provide greater efficiency than those hitherto used.

The lubricant medium envisaged in the present application is generally a petroleum oil or an emulsion thereof in water. Additives for securing particular properties in such lubricants have already been applied in the prior art in great variety. Such additives include compounds added to minimize metal-to-metal contact and the resulting damage to the metal under extreme conditions of pressure. Representative types of such compounds include sulphur compounds, halogen compounds and phosphorus compounds and substances in which these elements are combined, for instance organic sulphides and polysulphides and phospho-sulphurized compounds. Further examples are chlorinated kerosenes and chlorinated waxes. Another class of such additives includes sulphurized fats, fatty acids, esters and higher alcohols.

In very severe operations in which lubricants are used, for example broaching, a high proportion of additive is found to be necessary and may, for instance in the case of chlorinated wax, exceed 50 percent of the lubricant. Such a high proportion of additive material is inconvenient, costly and not always satisfactory from the point of view of the lubricant properties as such. Again, the sulphur frequently used in extreme pressure lubricants to impart anti-welding characteristics, may be required in a proportion or degree of activity sufficient to introduce corrosion of lubricated metal. Fatty oils and sulphurized fats in particular are unstable of themselves and lead to thickening of the oils and the development of unpleasant odour.

It is an object of the present invention to provide a compounded lubricating oil having unusual properties for metal cutting, metal rolling and particularly for cold rolling aluminum.

We have found that this and other objects of the invention are achieved compounding a highly chlorinated polyolefine and particularly a chlorinated polyolefine of a molecular weight range of about 50-1000 and a degree of chlorination of 20-60% by weight with a suitable base petroleum oil. The preferred molecular weight range of the polypropylene is 126 to 210 and the preferred chlorine content is 30 to 50% by weight of the product.

According to the present invention a compounded lubricating oil particularly useful for broaching, cutting and rolling is formed by adding to a lubricating oil of viscosity range 50-350 at 100° F. (S.U.S.) a small amount of a chlorinated polypropylene, such as Anchor N55 (trade name for polypropylene having a molecular weight of about 126 to 210 which is chlorinated to a chlorine content of about 30-50% by weight), wherein the poly-

2

propylene has a molecular weight of about 126-210 and is chlorinated to a chlorine content of about 30-50% by weight, manufactured and sold in Great Britain by the Anchor Chemical Company. A sulphurized mineral oil or sulphurized fatty oil may also be present and, if desired, an emulsifier. The preferred lubricating compound also contains a chlorinated wax, such as a chlorinated petroleum wax, either of the paraffin or microcrystalline type. The chlorinated wax, however, may vary quite widely provided it has a minimum chlorine content of 40% by weight. Such a wax is marketed in Great Britain by L.C.I. Limited under the trade name "Cereclor 42." The total amount of chlorinated additives including the chlorinated olefine and the chlorinated wax should amount to between 0.5% and 50% by weight of the total composition, preferably between 2% and 15%.

The sulphurized mineral oil is of the type already known for the purpose and may contain about 1% reactive sulphur as measured by the Institute of Petroleum test 155/58T "Sulphur (reactive to copper) in Cutting Oils." The proportion of sulphurized mineral oil is preferably less than 50% by weight of the total composition. The sulphurized fatty oil is also of the type known in the art and may be an animal or vegetable oil containing after sulphurization up to 20% sulphur in such a manner that the sulphur is largely unreactive to copper. The proportion of sulphurized fatty oil should preferably be limited to not more than 15% by weight of the composition.

30 The components other than the chlorinated polyolefine are of types generally known in the art and they may be varied in a manner known in principle to suit the severity of the lubricating operation for which they are intended. For instance, in the lubrication of heavy machinery, an oil of a suitable viscosity will be chosen and the proportions and selection of additive components made to suit the severity encountered, to provide, say, a "straight" cutting oil. In rolling or the machining of light metals on the other hand, where cooling is an important factor, an aqueous emulsion may be preferred.

35 The emulsifiers are of a conventional type, such as alkali metal petroleum sulphonates, alkali metal or alkaline earth metal soaps of naphthenic or rosin acids, and also so-called non-ionic emulsifiers.

40 45 Further additions may be made as desired, to modify the properties of the lubricating oil, such as fatty oils, fatty acids, esters, alcohols, polyglycols and their esters, antioxidants, anticorrosives, foam suppressors and bactericides. Coupling agents such as phenolic compounds and polyhydric alcohols may also be necessary.

50 55 The chlorinated polyolefine under the conditions of the test hereinafter described is more effective in preventing wear than the chlorinated wax at equal concentration. It has surprisingly been found, furthermore, that there is a synergistic effect between these additives in that part of the chlorinated olefine can be replaced by a similar amount of the chlorinated wax, the effectiveness of the combination being maintained at a higher level than is to be expected from proportionality, so long as the ratio of chlorinated polyolefine to chlorinated wax is not less than about 1:1, preferably 2:1. This is important economically at the higher additive concentrations where a considerable cost reduction can be effected by this means.

60 65 The interaction between the two chlorinated additives

was indicated by statistical analysis of the results of Falex and 4-ball wear tests on a set of experimental compositions designed on the fractional replicate principle. The interaction was seen to hold for the chlorinated additives alone and also in the presence of the sulphurized additives and a synergistic interaction was also indicated between the chlorinated additives and the sulphurized additives. These effects are illustrated in the accompanying tables showing the anti-wear properties of various compositions as measured by the 4-ball machine. In this test three steel balls are rigidly clamped in contact with each other and pressed by means of a loading lever against a rotating fourth steel ball which makes contact with all three stationary balls, the points of contact being lubricated by the composition under test. At fixed load, speed and time of rotation the average diameter of the scars left on the three stationary balls is a measure of the wear permitted by the lubricant and therefore the smaller the scar diameter the better the wear-preventing properties of the lubricant. The relative effects hold for a range of loads and can be illustrated by the results at one load.

4-ball tests in these cases were made on emulsions containing 10% of the oil and 90% of water by volume:

|                                          | D       | E       | F       | G               | H       |
|------------------------------------------|---------|---------|---------|-----------------|---------|
|                                          | Percent | Percent | Percent | Percent         | Percent |
| 5 Chlorinated Polypropylene (Anchor N55) | 2.0     |         | 5.0     |                 | 5.0     |
| Sodium Petroleum Sulphonates             | 5.0     |         |         | 5.0             | 5.0     |
| (Renex 688) Described below              |         | 5.0     | 4.75    |                 |         |
| 10 (Renex 697) Described below           | 6.0     | 5.0     | 4.75    | 6.0             | 6.0     |
| (Ethylan BCP) Described below            | 6.0     |         |         | 6.0             | 6.0     |
| Polyethylene glycol (300) di-oleate      | 5.0     | 14.0    | 13.30   | 5.0             | 5.0     |
| Rapeseed Oil                             | 5.0     | 5.0     | 4.75    | 5.0             | 5.0     |
| 15 Petroleum Oil, 100° S.U.V., 100° F    | 71.0    | 71.0    | 67.45   | 73.0            | 68.0    |
| Load, kg:                                |         |         |         | Ssar dia. (mm.) |         |
| 80                                       |         |         |         | 2.55            | 0.50    |
| 90                                       |         |         |         | 2.65            | 0.54    |
| 100                                      |         |         |         | Seized          | 0.57    |
|                                          |         |         |         | Seized          | Seized  |

Table I

| Chlorinated Polyolefine, Percent, Anchor N55 | Chlorinated Wax, Percent, Cereclor 42 | Petroleum Oil, Percent, Refined naphthenic oil of the Saybolt Universal Viscosity 100 sec. at 100° F. | Sulphurized Mineral Oil, Percent, Sulphurized fatty oil of minimum sulphur content 9% by weight | Sulphurized Fatty Oil, Percent (Sulphurized lard oil up to 1% reactive S, 100 seconds viscosity) | Scar Diameter (cm.) at load of— |         |
|----------------------------------------------|---------------------------------------|-------------------------------------------------------------------------------------------------------|-------------------------------------------------------------------------------------------------|--------------------------------------------------------------------------------------------------|---------------------------------|---------|
|                                              |                                       |                                                                                                       |                                                                                                 |                                                                                                  | 150 kg.                         | 300 kg. |
| 6                                            | —                                     | 94                                                                                                    | —                                                                                               | —                                                                                                | 0.077                           | —       |
| 5                                            | 1                                     | 94                                                                                                    | —                                                                                               | —                                                                                                | 0.086                           | —       |
| 3                                            | 3                                     | 94                                                                                                    | —                                                                                               | —                                                                                                | 0.086                           | —       |
| 1                                            | 5                                     | 94                                                                                                    | —                                                                                               | —                                                                                                | 0.124                           | —       |
| —                                            | 6                                     | 94                                                                                                    | —                                                                                               | —                                                                                                | 0.149                           | —       |
| 6                                            | —                                     | 64                                                                                                    | 30                                                                                              | —                                                                                                | —                               | 0.097   |
| 5                                            | 1                                     | 64                                                                                                    | 30                                                                                              | —                                                                                                | —                               | 0.100   |
| 3                                            | 3                                     | 64                                                                                                    | 30                                                                                              | —                                                                                                | —                               | 0.119   |
| 1                                            | 5                                     | 64                                                                                                    | 30                                                                                              | —                                                                                                | —                               | 0.131   |
| —                                            | 6                                     | 64                                                                                                    | 30                                                                                              | —                                                                                                | —                               | 0.153   |
| —                                            | —                                     | 70                                                                                                    | 30                                                                                              | —                                                                                                | —                               | 0.166   |
| 6                                            | —                                     | 91                                                                                                    | —                                                                                               | 3                                                                                                | —                               | 0.129   |
| 5                                            | 1                                     | 91                                                                                                    | —                                                                                               | 3                                                                                                | —                               | 0.134   |
| 3                                            | 3                                     | 91                                                                                                    | —                                                                                               | 3                                                                                                | —                               | 0.140   |
| 1                                            | 5                                     | 91                                                                                                    | —                                                                                               | 3                                                                                                | —                               | 0.226   |
| —                                            | 6                                     | 91                                                                                                    | —                                                                                               | 3                                                                                                | —                               | 0.224   |
| —                                            | —                                     | 97                                                                                                    | —                                                                                               | 3                                                                                                | —                               | Seized  |

The following table gives examples of straight metal working oils showing the corresponding 4-ball wear test results ("S.U.V." refers to second Saybolt Universal viscosity):

Table II

|                                        | A       | B       | C               |
|----------------------------------------|---------|---------|-----------------|
|                                        | Percent | Percent | Percent         |
| Chlorinated polypropylene (Anchor N55) | 2.0     | 10.0    | 4.0             |
| Chlorinated wax (Cereclor 42)          | —       | 5.0     | —               |
| Sulphurized petroleum oil              | 30.0    | —       | 30.0            |
| Dioleyl Malate                         | 0.5     | 0.5     | 0.5             |
| Petroleum Lubricating Oil:             |         |         |                 |
| 55° S.U.V. at 100° F.                  | —       | 84.5    | —               |
| 100° S.U.V. at 100° F.                 | 67.5    | —       | —               |
| 220° S.U.V. at 100° F.                 | —       | —       | 65.5            |
| Load, kg:                              |         |         |                 |
|                                        |         |         | Scar dia. (mm.) |
| 150                                    | 0.82    | 0.66    | —               |
| 250                                    | 1.23    | 0.91    | —               |
| 350                                    | 1.51    | 1.30    | 1.17            |
| 450                                    | 1.66    | 1.58    | 1.42            |
| 500                                    | 1.83    | 1.68    | 1.46            |
| 600                                    | Seized  | 1.94    | 1.60            |
| 700                                    | —       | —       | 1.73            |

The following table gives examples of soluble oils.

The sulphonates are sodium petroleum mahogany sulphonates of molecular weight about 420.

50 The "Renex" and "Ethylan" materials are condensation products of nonyl-phenol with ethylene oxide. The nonyl-phenol used in the preparation of these materials is a mixture of ortho- and para-nonyl phenol in which the para-isomer predominates in the proportion of about 85 parts to 15 parts of the ortho. In Renex 688, Renex 697, and Ethylan BCP one mol. of the nonyl-phenol is condensed with 8, 6 and 9 mols respectively of ethylene oxide.

The polyethylene glycol (300) di-oleate is the di-oleate ester of a polyethylene glycol of molecular weight approximately 300.

The examples given hereinabove are supplied to illustrate the invention without in any way limiting the scope of the invention. The only limitations intended are those found in the attached claim.

65 We claim:

A lubricating composition comprising (1) a major proportion of a petroleum lubricating oil having a viscosity in the range of 50-350 S.U.V. at 100° F., (2) a minor proportion of a sulphurized mineral oil, (3) about 2-15% by weight of a chlorinated petroleum wax having a chlorine content of at least 40% by weight, and (4) about 2-15% by weight of a chlorinated polypropylene, the polypropylene having a molecular weight of about 126-210 and being chlorinated to a chlorine content of about

30-50% by weight, said composition being further characterized in that the ratio of the chlorinated polypropylene to the chlorinated petroleum wax is at least 2:1.

**References Cited** in the file of this patent

**UNITED STATES PATENTS**

|           |               |                |           |
|-----------|---------------|----------------|-----------|
| 2,126,590 | Valentine     | Aug. 9, 1938   | 2,403,179 |
| 2,225,318 | Morway et al. | Dec. 17, 1940  | 2,621,159 |
| 2,296,037 | Kaufman       | Sept. 15, 1942 | 2,682,523 |
| 2,298,833 | Muessig       | Oct. 13, 1942  | 2,848,416 |

5

2,852,468  
2,921,903  
2,993,857  
10      569,348

Hull et al. July 2, 1946  
Perry et al. Dec. 9, 1952  
Talley et al. June 29, 1954  
Gililland et al. Aug. 19, 1958  
Hughes et al. Sept. 16, 1958  
Beretvas Jan. 19, 1960  
Sudholz July 25, 1961

**FOREIGN PATENTS**

Great Britain May 18, 1945